

# United States Patent [19]

Price

[11] 3,964,912

[45] June 22, 1976

[54] RUTHENIUM CONTAINING  
PHOTOGRAPHIC DEVELOPERS

3,765,891 10/1973 Travis ..... 96/55  
3,862,842 1/1975 Bissonette ..... 96/66 R

[75] Inventor: Harry J. Price, Rochester, N.Y.

Primary Examiner—Mary F. Kelley  
Attorney, Agent, or Firm—Carl O. Thomas

[73] Assignee: Eastman Kodak Company,  
Rochester, N.Y.

[22] Filed: Dec. 29, 1975

## [57] ABSTRACT

[21] Appl. No.: 645,104

A composition is disclosed useful in developing silver halide photographic elements containing specifically selected developing agents for silver halide and a ruthenium(II) or ruthenium(III) cationic complex as a development accelerator. The ruthenium complex includes a predominance of amine or ammine ligands. Each of the developing agents exhibits an induction period in the absence of the ruthenium complex in excess of about 5 seconds. Polyhydroxybenzene, ascorbic acid, hydroxylamine, hydroxyurea and pyrimidine developing agents are representative of those which are useful in the practice of my invention. A method of accelerating photographic development using the above composition is also disclosed.

### Related U.S. Application Data

[63] Continuation of Ser. No. 504,596, Sept. 9, 1974,  
abandoned, and a continuation-in-part of Ser. No.  
483,252, June 26, 1974, abandoned.

[52] U.S. Cl. .... 96/66.3; 96/66 HD;  
96/66 R

[51] Int. Cl.<sup>2</sup> .... G03C 5/30

[58] Field of Search .... 96/50, 63, 66, 66.3,  
96/95

### [56] References Cited

#### UNITED STATES PATENTS

3,748,138 7/1973 Bissonette ..... 96/66.3

24 Claims, No Drawings

## RUTHENIUM CONTAINING PHOTOGRAPHIC DEVELOPERS

This is a continuation of application Ser. No. 504,596, filed Sept. 9, 1974, and a continuation-in-part of my copending patent application Ser. No. 483,252, filed June 26, 1974, now abandoned.

My invention relates to novel photographic silver halide developers. More specifically, my invention relates to compositions useful in developing silver halide photographic elements which compositions contain at least one silver halide developing agent and a development accelerator.

I have discovered quite unexpectedly that when each of the developing agents present exhibit (in the absence of any other developing agents which may be present) an induction period in excess of 5 seconds, the performance of the developer can be significantly enhanced through the incorporation of at least one ruthenium(III) or (II) cationic complex which includes a predominance of ammine or amine ligands, provided at least one of the developing agents exhibits a rate of reduction of ruthenium(III) in the ruthenium(III) cationic complex, or produced by oxidation of the ruthenium(II) cationic complex, which exceeds its rate of reduction of silver halide.

In relation to photographic developers consisting essentially of polyhydroxybenzene, ascorbic acid, hydroxylamine, hydroxyurea and/or pyrimidine developing agents, I have discovered quite surprisingly that any cationic ruthenium(III) complex incorporated or produced in situ which exhibits a ruthenium(III) reduction potential no less positive than the oxidation potential of at least one of the developing agents will function as a development accelerator.

Stated in a different way, I have discovered that the development of silver halide photographic elements can be accelerated through the incorporation of ruthenium complexes in basic aqueous photographic developers where the ruthenium complexes and developing agents are as indicated above.

Based upon my knowledge of the state of the art at the time of my discovery I consider these novel photographic silver halide developers to be surprisingly advantageous. In the November-December 1970 issue of *Photographic Science and Engineering*, Vol. 14, No. 6, I published an article titled "The Mechanism of Development by Metal Complexes". In my article I reported observations based on the use of ruthenium(II) hexamine as a developing agent—not in combination with known developing agents, but as a sole developing agent.

Bissonnette, U.S. Pat. 3,748,138, issued July 24, 1973 (filed Oct. 14, 1971), commonly assigned, teaches the use of metal coordination complexes having a coordination number of 6—specifically, cobalt and chromium complexes—to be useful development accelerators either when incorporated into a silver halide emulsion or when employed in certain photographic developers. In Examples 1 through 3 Bissonnette employs hydroquinone, a developing agent having an induction period in excess of 5 seconds, in combination with N-methyl-p-aminophenol sulfate, a developing agent exhibiting an induction period substantially below 5 seconds (approximately 1 second at a pH of 10). In the remaining Examples each of the developing agents exhibit an induction period of less than 5 seconds. Except for the hydroquinone developing agent of Examples 1 through

3, every developing agent named by Bissonnette exhibits an induction period of well below 5 seconds and/or a reduction rate for silver halide which exceeds the rate at which it reduces ruthenium(III) cationic complexes.

5 It is therefore apparent that Bissonnette does not specifically disclose any photographic silver halide developer in which each developing agent present, in the absence of other developing agents, exhibits an induction period in excess of 5 seconds and in which at least one of the developing agents more readily reduces a ruthenium(II) cationic complex than silver halide. Further, Bissonnette does not specifically mention ruthenium complexes as being useful development accelerators.

10 Beavers U.S. Ser. No. 398,515, filed Sept. 18, 1973, commonly assigned, which is a continuation-in-part of Beavers U.S. Ser. No. 312,159, filed Dec. 4, 1972, now abandoned, teaches the incorporation of cobalt(III) and chromium(III) ammine and amine complexes in photographic silver halide emulsions in combination with azaindene anti-foggers.

15 In *Research Disclosure*, Vol. 109, pp. 28-31, Item 10908, titled "Lithographic Materials Containing Metal Complexes," published May 1973, it is disclosed to incorporate cobalt(III) and chromium(III) complexes containing certain ammine and amine ligands into silver halide emulsions for the purpose of accelerating development. A hydroquinone "lith-type" developer (Developer A in Masseth U.S. Pat. 3,573,914, issued Apr. 6, 1971) is employed. Ruthenium(III) complexes are reported to have been tested under conditions similar to those employed in testing the cobalt(III) and chromium(III) complexes, but the contrasts achieved were too low for use in lithographic type photographic elements. In Beavers U.S. Ser. No.

20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9

tographic developers containing cobalt(III) and chromium(III) ammine and amine ligand complexes as development accelerators were found to require a significant degree of care in storage and use.

This then was the state of the art when Beavers discovered significant advantages for incorporating cobalt(III) and chromium(II) complexes in photographic silver halide emulsions in combination with azaindene anti-foggants. The combination of ruthenium(III) complexes with azaindenes at like concentrations in emulsions did not, however produce corresponding advantages. Beavers' later discovery that ruthenium complexes at concentrations below 1 gram per mole of silver could be advantageously incorporated in photographic silver halide emulsions was not known to me at the time of my invention.

I have discovered quite unexpectedly that ruthenium(II) and (III) cationic complexes having a predominance of ammine and amine ligands can be employed to reduce the induction period of certain types of developing agents having substantial induction periods—that is, in excess of about 5 seconds. I have found that induction periods can be decreased in most instances by approximately an order of magnitude. I have further observed that these ruthenium complexes in combination with such developing agents significantly increase that rate of development following the induction period—i.e., the continuation stage of development.

I have additionally observed that these ruthenium complexes offer distinct advantages over corresponding cobalt(III) and chromium(III) complexes. First, I have observed that both ruthenium(III) and ruthenium(II) complexes can be employed advantageously in the practice of my invention. Whereas the effectiveness of cobalt(III) and chromium(III) complexes is destroyed by ligand release in reduction to cobalt(II) and chromium(II) complexes, ruthenium(III) complexes do not lose ligands or effectiveness by reduction to ruthenium(II) complexes. This then overcomes one of the principal disadvantages that have been encountered in using metal complexes of this type as development accelerators in photographic silver halide developers. For reasons more fully discussed below, this also permits comparatively lower concentrations of ruthenium complexes to be employed. I have further observed combinations of ruthenium complexes and developing agents according to my invention to form more effective photographic silver halide developers than corresponding combinations including either cobalt(III) or chromium(III) complexes. I also believe that the various advantages for the use of ruthenium complexes in photographic silver halide emulsions set forth in Beavers U.S. Ser. No. 450,263, cited above, could also be achieved in the practice of my invention.

While I do not wish to be bound by any particular theory, it is my belief that ruthenium complexes function as development accelerators in the photographic silver halide developers of my invention in a manner that differs markedly from that of corresponding cobalt(III) and chromium(III) development accelerators. In considering a photographic silver halide developer containing a ruthenium complex development accelerator and a developing agent which requires a substantial induction period in the absence of the ruthenium complex and which more readily reduces ruthenium(III) than silver halide, it is my belief that the ruthenium complex forms a redox couple between the developing agent and the silver halide. That is, a continuous

cycling of the ruthenium complex occurs between (1) an oxidation-reduction reaction with the developing agent in which the ruthenium is reduced from ruthenium(III) to ruthenium(II) while the developing agent is oxidized and (2) an oxidation-reduction reaction with silver halide in which the ruthenium(II) is oxidized and silver halide is reduced to metallic silver to form a silver image. In these reactions the ruthenium complex acts as a catalyst for development of silver halide and is not consumed. Thus, low concentrations of ruthenium are effective. It is also apparent that corresponding ruthenium(III) and (II) complexes can be employed interchangeably, since it is immaterial whether the ruthenium complex first oxidizes the developing agent or reduces silver halide.

These and other advantageous features of my invention will become further apparent in the following description of certain preferred embodiments.

The cationic ruthenium complexes employed in the practice of this invention comprise a divalent or trivalent ruthenium ion surrounded by certain other molecules which are referred to as ligands. The ruthenium ion is a Lewis acid; the ligands are Lewis bases. Werner complexes are well known examples of these complexes. While it is possible to form ruthenium complexes that are neutral (i.e., carry no net charge) or are negatively charged, only ruthenium complexes exhibiting a net positive charge, i.e., cationic complexes, are employed in the practice of this invention.

The cationic ruthenium complexes employed in the practice of this invention include a predominance of (that is, at least four) ammine or amine ligand coordination bonds. The amine ligands include primary, secondary and tertiary amine ligands and include diamines and heterocyclic amines. One preferred class of amine ligands are acyclic aliphatic amine ligands, such as those comprised of alkyl, alkylene and alkanol aliphatic moieties. Each aliphatic moiety preferably includes 6 or fewer carbon atoms. Alkylene diamines have been found particularly useful in forming bidentate ligands.

Bidentate ligands which form with the ruthenium atom 5- to 8-membered rings have been found to produce particularly stable complexes. Typical heterocyclic amine ligands and comprised of 5- and 6-membered rings including at least one nitrogen atom with the remaining atoms being entirely carbon atoms or including at most one other hetero atom, such as nitrogen, oxygen, or sulfur. Exemplary preferred ammine and amine ligand-forming compounds include ammonia, ethylene diamine, trimethylene diamine, diethanol amine, diopropanol amine, diethylene triamine, alkyltetramines, pyridine, morpholine, pyrrole, pyrazole, pyrazine, pyrazoline, oxazole, thiazole, etc.

A minor proportion of the coordination bonds making up the cationic ruthenium complex can be provided by ligands other than ammine or amine ligands. A ruthenium(II) or (III) complex can contain 1 or 2 monodentate ligands, such as water, halogen, thiocyanate, etc., or a single bidentate ligand.

There will, of course, be anions associated with the foregoing complex cations. Any anion which does not exert undesirable effects upon the photographic element being processed may be employed. Typical useful anions include chloride, bromide, sulfite, sulfate, perchlorate, nitrite, nitrate, tetrabromozincate, tetrafluoroborate, hexafluorophosphate, thiocyanate, dithionite, methyl sulfonate, tolyl sulfonate, and the like.

While a variety of ruthenium(II) and (III) complexes can be employed in the practice of my invention, for any specific application the choice of a ruthenium complex must be considered in conjunction with the choice of developing agent. To assure that at least one developing agent exhibits a rate of reduction of the ruthenium(III) complex in the photographic silver halide developer which exceeds the rate at which it directly reduces silver halide in the absence of the ruthenium(III) complex, the ruthenium(III) complex is chosen to have a reduction potential which at least equals or is more positive than the oxidation potential of the developing agent. In a preferred form of the invention the ruthenium(III) complex present in the photographic silver halide developer exhibits a reduction potential which is intermediate between the oxidation potential of the developing agent and the reduction potential of the silver halide being developed. For example, where hydroquinone is being employed as the developing agent for silver bromide, the ruthenium(III) complex preferably exhibits a reduction potential between 0.10 volt, the oxidation potential of hydroquinone, and 0.70 volt, the reduction potential of silver bromide.

Exemplary of ruthenium(II) and (III) complexes useful in the practice of this invention are those set forth below in Table I. The reduction potentials of the ruthenium(III) complexes are measured by the procedures set forth by Lim, Barclay and Anson, *Inorganic Chemistry*, Vol. 11, No. 7, "Formal Potentials and Cyclic Voltammetry of Some Ruthenium-Ammine Complexes", 1972. It can be seen that the selection of the anion associated with the complex does not affect its reduction potential.

TABLE I

| Exemplary Cationic Ruthenium Complexes |                                               |
|----------------------------------------|-----------------------------------------------|
| RU- 1a                                 | hexammine ruthenium(III) chloride             |
| RU- 1b                                 | hexammine ruthenium(II) chloride              |
| RU- 2a                                 | hexammine ruthenium(III) bromide              |
| RU- 2b                                 | hexammine ruthenium(II) bromide               |
| RU- 3a                                 | hexammine ruthenium(III) sulfite              |
| RU- 3b                                 | hexammine ruthenium(II) sulfite               |
| RU- 4a                                 | hexammine ruthenium(III) perchlorate          |
| RU- 4b                                 | hexammine ruthenium(II) perchlorate           |
| RU- 5a                                 | hexammine ruthenium(III) nitrate              |
| RU- 5b                                 | hexammine ruthenium(II) nitrate               |
| RU- 6a                                 | hexammine ruthenium(III) hexafluorophosphate  |
| RU- 6b                                 | hexammine ruthenium(II) hexafluorophosphate   |
| RU- 7a                                 | hexammine ruthenium(III) thiocyanate          |
| RU- 7b                                 | hexammine ruthenium(II) thiocyanate           |
| RU- 8a                                 | hexammine ruthenium(III) methylsulfonate      |
| RU- 8b                                 | hexammine ruthenium(II) methylsulfonate       |
| RU- 9a                                 | tris(ethylenediamine) ruthenium-(III) bromide |
| RU- 9b                                 | tris(ethylenediamine) ruthenium-(II) bromide  |
| RU-10a                                 | tris(ethylenediamine) ruthenium-(III) sulfate |
| RU-10b                                 | tris(ethylenediamine) ruthenium-              |

|    |        | Exemplary Cationic Ruthenium Complexes                      | Reduction Potentials (volts) for Ruthenium (III) Complexes |
|----|--------|-------------------------------------------------------------|------------------------------------------------------------|
| 5  |        |                                                             |                                                            |
| 10 | RU-11a | (II) sulfate<br>tris(ethylenediamine) ruthenium-            | +0.20                                                      |
|    | RU-11b | (III) nitrate<br>tris(ethylenediamine) ruthenium-           |                                                            |
|    | RU-12a | (II) nitrate<br>tris(ethylenediamine) ruthenium-            | +0.20                                                      |
|    | RU-12b | (III) tetrabromozincate<br>tris(ethylenediamine) ruthenium- |                                                            |
| 15 | RU-13a | (II) tetrabromozincate<br>tris(ethylenediamine) ruthenium-  |                                                            |
|    | RU-13b | (III) tetrafluoroborate<br>tris(ethylenediamine) ruthenium- | +0.20                                                      |
|    | RU-14a | (II) tetrafluoroborate<br>tris(ethylenediamine) ruthenium-  |                                                            |
|    | RU-14b | (III) thiocyanate<br>tris(ethylenediamine) ruthenium-       | +0.20                                                      |
| 20 | RU-15a | (II) thiocyanate<br>tris(ethylenediamine) ruthenium-        |                                                            |
|    | RU-15b | (III) methylsulfonate<br>tris(ethylenediamine) ruthenium-   | +0.20                                                      |
|    | RU-16a | (II) methylsulfonate<br>tris(ethylenediamine) ruthenium-    |                                                            |
|    | RU-16b | (III) tolylsulfonate<br>tris(ethylenediamine) ruthenium-    | +0.20                                                      |
| 25 | RU-17a | (II) tolylsulfonate<br>monochloropentammine ruthenium-      |                                                            |
|    | RU-17b | (III) chloride<br>monochloropentammine ruthenium-           | -0.042                                                     |
|    | RU-18a | (II) chloride<br>monochloropentammine ruthenium-            |                                                            |
| 30 | RU-18b | (III) nitrite<br>monochloropentammine ruthenium-            | -0.042                                                     |
|    | RU-19a | (II) nitrite<br>monochloropentammine ruthenium-             |                                                            |
|    | RU-19b | (III) nitrate<br>monochloropentammine ruthenium-            | -0.042                                                     |
|    | RU-20a | (II) nitrate<br>monochloropentammine ruthenium-             |                                                            |
| 35 | RU-20b | (III) tetrabromozincate<br>monochloropentammine ruthenium-  | -0.042                                                     |
|    | RU-21a | (II) tetrabromozincate<br>monochloropentammine ruthenium-   |                                                            |
|    | RU-21b | (III) sulfate<br>monochloropentammine ruthenium-            | -0.42                                                      |
| 40 | RU-22a | (II) sulfate<br>monochloropentammine ruthenium-             |                                                            |
|    | RU-22b | (III) perchlorate<br>monochloropentammine ruthenium-        | -0.042                                                     |
|    | RU-23a | (II) perchlorate<br>monochloropentammine ruthenium-         |                                                            |
|    | RU-23b | (III) thiocyanate<br>monochloropentammine ruthenium-        | -0.042                                                     |
| 45 | RU-24a | (II) thiocyanate<br>monochloropentammine ruthenium-         |                                                            |
|    | RU-24b | (III) dithionate<br>monochloropentammine ruthenium-         | -0.042                                                     |
|    | RU-25a | (II) dithionate<br>bromopentammine ruthenium(III)           |                                                            |
| 50 | RU-25b | bromide<br>bromopentammine ruthenium(II)                    | -0.03                                                      |
|    | RU-26a | bromide<br>bromopentammine ruthenium(III)                   |                                                            |
|    | RU-26b | sulfite<br>bromopentammine ruthenium(II)                    | -0.03                                                      |
|    | RU-27a | sulfite<br>bromopentammine ruthenium(III)                   |                                                            |
| 55 | RU-27b | nitrite<br>bromopentammine ruthenium(II)                    | -0.03                                                      |
|    | RU-28a | nitrite<br>bromopentammine ruthenium(III)                   |                                                            |
|    | RU-28b | tetrabromozincate<br>bromopentammine ruthenium(II)          | -0.03                                                      |
| 60 | RU-28b | tetrabromozincate<br>bromopentammine ruthenium(III)         |                                                            |
|    | RU-29b | tetrafluoroborate<br>bromopentammine ruthenium(II)          | -0.03                                                      |
|    | RU-30a | tetrafluoroborate<br>bromopentammine ruthenium(III)         |                                                            |
|    | RU-30b | hexafluorophosphate<br>bromopentammine ruthenium(II)        | -0.03                                                      |
| 65 | RU-31a | hexafluorophosphate<br>bromopentammine ruthenium(III)       |                                                            |
|    | RU-31b | dithionate<br>bromopentammine ruthenium(II)                 | -0.03                                                      |
|    | RU-32a | dithionate<br>bromopentammine ruthenium(III)                |                                                            |

TABLE I-continued

|        | Exemplary Cationic Ruthenium Complexes                                 | Reduction Potentials (volts) for Ruthenium(III) Complexes | 5  |
|--------|------------------------------------------------------------------------|-----------------------------------------------------------|----|
| RU-32b | tolyl sulfonate bromopentammine ruthenium(III)                         | -0.03                                                     |    |
| RU-33a | tolyl sulfonate diaquotetrammine ruthenium(III) chloride               | +0.10                                                     | 10 |
| RU-33b | tolyl sulfonate diaquotetrammine ruthenium(II) chloride                | +0.10                                                     |    |
| RU-34a | tolyl sulfonate diaquotetrammine ruthenium(III) sulfite                | +0.10                                                     | 15 |
| RU-34b | tolyl sulfonate diaquotetrammine ruthenium(II) sulfite                 | +0.10                                                     |    |
| RU-35a | tolyl sulfonate diaquotetrammine ruthenium(III) sulfate                | +0.10                                                     |    |
| RU-35b | tolyl sulfonate diaquotetrammine ruthenium(II) sulfate                 | +0.10                                                     |    |
| RU-36a | tolyl sulfonate diaquotetrammine ruthenium(III) perchlorate            | +0.10                                                     | 20 |
| RU-36b | tolyl sulfonate diaquotetrammine ruthenium(II) perchlorate             | +0.10                                                     |    |
| RU-37a | tolyl sulfonate diaquotetrammine ruthenium(III) nitrite                | +0.10                                                     |    |
| RU-37b | tolyl sulfonate diaquotetrammine ruthenium(II) nitrite                 | +0.10                                                     |    |
| RU-38a | tolyl sulfonate diaquotetrammine ruthenium(III) tetrafluoroborate      | +0.10                                                     | 25 |
| RU-38b | tolyl sulfonate diaquotetrammine ruthenium(II) tetrafluoroborate       | +0.10                                                     |    |
| RU-39a | tolyl sulfonate diaquotetrammine ruthenium(III) methylsulfonate        | +0.10                                                     |    |
| RU-39b | tolyl sulfonate diaquotetrammine ruthenium(II) methylsulfonate         | +0.10                                                     |    |
| RU-40a | tolyl sulfonate diaquotetrammine ruthenium(III) tolylsulfonate         | +0.10                                                     | 30 |
| RU-40b | tolyl sulfonate diaquotetrammine ruthenium(II) tolylsulfonate          | +0.10                                                     |    |
| RU-41a | tolyl sulfonate pyridine pentammine ruthenium(III) sulfite             | +0.30                                                     |    |
| RU-41b | tolyl sulfonate pyridine pentammine ruthenium(II) sulfite              | +0.30                                                     | 35 |
| RU-42a | tolyl sulfonate pyridine pentammine ruthenium(III) sulfate             | +0.30                                                     |    |
| RU-42b | tolyl sulfonate pyridine pentammine ruthenium(II) sulfate              | +0.30                                                     |    |
| RU-43a | tolyl sulfonate pyridine pentammine ruthenium(III) hexafluorophosphate | +0.30                                                     |    |
| RU-43b | tolyl sulfonate pyridine pentammine ruthenium(II) hexafluorophosphate  | +0.30                                                     | 40 |
| RU-44a | tolyl sulfonate pyridine pentammine ruthenium(III) dithionate          | +0.30                                                     |    |
| RU-44b | tolyl sulfonate pyridine pentammine ruthenium(II) dithionate           | +0.30                                                     |    |
| RU-45a | tolyl sulfonate pyridine pentammine ruthenium(III) methyl sulfonate    | +0.30                                                     | 45 |
| RU-45b | tolyl sulfonate pyridine pentammine ruthenium(II) methyl sulfonate     | +0.30                                                     |    |
| RU-46a | tolyl sulfonate pyrazine pentammine ruthenium(III) bromide             | +0.49                                                     |    |
| RU-46b | tolyl sulfonate pyrazine pentammine ruthenium(II) bromide              | +0.49                                                     | 50 |
| RU-47a | tolyl sulfonate pyrazine pentammine ruthenium(III) perchlorate         | +0.49                                                     |    |
| RU-47b | tolyl sulfonate pyrazine pentammine ruthenium(II) perchlorate          | +0.49                                                     |    |
| RU-48a | tolyl sulfonate pyrazine pentammine ruthenium(III) tetrabromozincate   | +0.49                                                     | 55 |
| RU-48b | tolyl sulfonate pyrazine pentammine ruthenium(II) tetrabromozincate    | +0.49                                                     |    |
| RU-49a | tolyl sulfonate pyrazine pentammine ruthenium(III) tetrafluoroborate   | +0.49                                                     |    |
| RU-49b | tolyl sulfonate pyrazine pentammine ruthenium(II) tetrafluoroborate    | +0.49                                                     |    |
| RU-50a | tolyl sulfonate pyrazine pentammine ruthenium(III) thiocyanate         | +0.49                                                     | 60 |
| RU-50b | tolyl sulfonate pyrazine pentammine ruthenium(II) thiocyanate          | +0.49                                                     |    |
| RU-51a | tolyl sulfonate pyrazine pentammine ruthenium(III) tolyl sulfonate     | +0.49                                                     |    |
| RU-51b | tolyl sulfonate pyrazine pentammine ruthenium(II) tolyl sulfonate      | +0.49                                                     |    |
| RU-52a | tolyl sulfonate pyrazine pentammine ruthenium(III) chloride            | +0.44                                                     | 65 |
| RU-52b | tolyl sulfonate pyrazine pentammine ruthenium(II) chloride             | +0.44                                                     |    |
| RU-53a | tolyl sulfonate pyrazine pentammine ruthenium(III) nitrite             | +0.44                                                     |    |
| RU-53b | tolyl sulfonate pyrazine pentammine ruthenium(II) nitrite              | +0.44                                                     |    |

TABLE I-continued

|        | Exemplary Cationic Ruthenium Complexes                                  | Reduction Potentials (volts) for Ruthenium(III) Complexes |
|--------|-------------------------------------------------------------------------|-----------------------------------------------------------|
| RU-54a | ruthenium(II) nitrite isonicotinamido pentammine ruthenium(III) nitrate | +0.44                                                     |
| RU-54b | isonicotinamido pentammine ruthenium(II) nitrate                        |                                                           |
| RU-55a | isonicotinamido pentammine ruthenium(III) dithionate                    | +0.44                                                     |
| RU-55b | isonicotinamido pentammine ruthenium(II) dithionate                     |                                                           |
| RU-56a | 4-(methylcarboxylato)pyridine pentammine ruthenium(III) bromide         | +0.46                                                     |
| RU-56b | 4-(methylcarboxylato)pyridine pentammine ruthenium(II) bromide          |                                                           |
| RU-57a | 4-(methylcarboxylato)pyridine pentammine ruthenium(III) sulfite         | +0.46                                                     |
| RU-57b | 4-(methylcarboxylato)pyridine pentammine ruthenium(II) sulfite          |                                                           |
| RU-58a | 4-(methylcarboxylato)pyridine pentammine ruthenium(III) sulfate         | +0.46                                                     |
| RU-58b | 4-(methylcarboxylato)pyridine pentammine ruthenium(II) sulfate          |                                                           |
| RU-59a | 4-(methylcarboxylato)pyridine pentammine ruthenium(III) perchlorate     | +0.46                                                     |
| RU-59b | 4-(methylcarboxylato)pyridine pentammine ruthenium(II) perchlorate      |                                                           |
| RU-60a | 4-(methylcarboxylato)pyridine pentammine ruthenium(III) nitrite         | +0.46                                                     |
| RU-60b | 4-(methylcarboxylato)pyridine pentammine ruthenium(II) nitrite          |                                                           |
| RU-61a | 4-(methylcarboxylato)pyridine pentammine ruthenium(III) nitrate         | +0.46                                                     |
| RU-61b | 4-(methylcarboxylato)pyridine pentammine ruthenium(II) nitrate          |                                                           |
| RU-62a | tris(2,2'-bipyridine) ruthenium(III) chloride                           | +1.20                                                     |
| RU-62b | tris(2,2'-bipyridine) ruthenium(II) chloride                            |                                                           |
| RU-63a | tris(2,2'-bipyridine) ruthenium(III) tetrabromozincate                  | +1.20                                                     |
| RU-63b | tris(2,2'-bipyridine) ruthenium(II) tetrabromozincate                   |                                                           |
| RU-64a | tris(2,2'-bipyridine) ruthenium(III) hexafluorophosphate                | +1.20                                                     |
| RU-64b | tris(2,2'-bipyridine) ruthenium(II) hexafluorophosphate                 |                                                           |
| RU-65a | tris(2,2'-bipyridine) ruthenium(III) dithionate                         | +1.20                                                     |
| RU-65b | tris(2,2'-bipyridine) ruthenium(II) dithionate                          |                                                           |

<sup>a</sup>Meyer and Taube, "Electron-Transfer Reaction of Ruthenium Ammines", Inorganic Chemistry, Vol. 7, No. 11, November, 1968.

Since the ruthenium complexes employed in the practice of this invention are not consumed in use, very low concentrations are effective. It is generally unnecessary to employ the ruthenium complexes in concentrations greater than 0.1 mole per liter of the photographic silver halide developer. It is generally preferred to use the ruthenium complexes in concentrations of from  $1 \times 10^{-5}$  to  $1 \times 10^{-3}$  moles per liter, although any development accelerating amount of the ruthenium complexes can be employed.

It is contemplated to employ the ruthenium complexes in photographic silver halide developers in which each of the developing agents present exhibits in the absence of other developing agents and the ruthenium complex a substantial induction period—e.g., in excess of about 5 seconds. The induction periods of most common photographic silver halide developing agents have been measured and reported in the literature. Alternately, the induction period for any given developing agent can be readily determined merely by formulating the developer with only that developing

agent present and the ruthenium complex absent and observing the development properties of the resulting photographic developer. The method for measuring the induction period of a developing agent and the development rate in the continuation stage is described in a paper by R. G. Willis and R. B. Pontius, *Photographic Science and Engineering*, Vol. 14, p. 385 (1970). FIG. 1 on page 387 of that paper is an example of the type of plot from which these values are determined.

In addition to exhibiting substantial induction periods at least one of the developing agents present is chosen to exhibit a rate of reduction of ruthenium(III) which exceeds its rate of reduction of silver halide. The ruthenium(III) reduced is that which is either in the ruthenium complex initially or which is formed by the oxidation of the ruthenium(II) in the complex. If a developing agent, such as 1-phenyl-3-pyrazolidone, dihydroanhydropiperidinohexose reductone, or 4-amino-N-ethyl-N-( $\beta$ -methanesulfonamidoethyl)-m-toluidine sesquisulfate, which exhibits no observable induction period even in the absence of a ruthenium complex, is employed, no development acceleration can be observed through the incorporation of a ruthenium(III) complex even though the developing agent may more readily reduce the ruthenium(III) complex than silver halide. On the other hand, in observing the behavior of developing agents, e.g., p-aminophenol and p-phenylenediamine color developing agents, having induction periods ranging from 1 second to well in excess of 5 seconds, but which more readily reduce silver halide than ruthenium(III) complexes, I have not observed development acceleration to occur, except when such developing agents are employed in combination with other developing agents which also have substantial induction periods and which exhibit a greater reduction rate for the ruthenium(III) complex present than for silver halide.

One preferred class of developing agents are polyhydroxybenzenes. I have found pyrogallols, catechols and hydroquinones to be particularly useful developing agents in the practice of my invention. Exemplary preferred polyhydroxybenzene developing agents are set forth in Table II.

TABLE II

| Exemplary Polyhydroxybenzene Developing Agents |                                                       |
|------------------------------------------------|-------------------------------------------------------|
| DA- 1                                          | catechol                                              |
| DA- 2                                          | gallic acid                                           |
| DA- 3                                          | phloroglucinol                                        |
| DA- 4                                          | pyrogallol                                            |
| DA- 5                                          | hydroxyhydroquinone                                   |
| DA- 6                                          | hydroquinone                                          |
| DA- 7                                          | chlorohydroquinone                                    |
| DA- 8                                          | bromohydroquinone                                     |
| DA- 9                                          | isopropylhydroquinone                                 |
| DA-10                                          | toluhydroquinone                                      |
| DA-11                                          | methylhydroquinone                                    |
| DA-12                                          | 2,3-dichlorohydroquinone                              |
| DA-13                                          | 2,5-dimethylhydroquinone                              |
| DA-14                                          | 2,3-dibromohydroquinone                               |
| DA-15                                          | 1,4-dihydroxy-2-acetophenone-2,5-dimethylhydroquinone |
| DA-16                                          | 2,5-diethylhydroquinone                               |
| DA-17                                          | 2,5-di-p-phenethylhydroquinone                        |
| DA-18                                          | 2,5-dibenzoylaminohydroquinone                        |
| DA-19                                          | 2,5-diacetaminohydroquinone                           |

Another preferred class of developing agents is comprised of hydroxylamine developing agents. Such developing agents are characterized by the hydroxy substituted nitrogen atom of the amine also being substi-

tuted with at least one organic aliphatic or aromatic radical. Such hydroxylamine developing agents include N-alkyl and N,N-dialkylhydroxylamines N-alkoxyalkyl and N,N-dialkoxyalkylhydroxylamines, N-arylhydroxylamines, N-alkarylhydroxylamines, etc. In each instance the alkyl moiety is preferably comprised of from 1 to 5 carbon atoms and the aryl moiety is preferably a phenyl moiety. Other hydroxylamine developing agents containing intralinear sulfo and intralinear cyclic or acyclic nitrogen atoms are disclosed in U.S. Pats. 3,287,124 and 3,287,125, each issued Nov. 22, 1966. Other hydroxylamine developing agents are disclosed in U.S. Pats. 2,857,274; 2,857,275 and 2,857,276, each issued Oct. 21, 1958; in British Patent 1,142,134, published Feb. 5, 1969, and in Belgium Patent 558,501, published July 15, 1957. The use of cyclic hydroxylamines, such as N-hydroxymorpholine, is also contemplated.

Exemplary preferred hydroxylamine developing agents are set forth below in Table III.

TABLE III

| Exemplary Hydroxylamine Developing Agents |                                   |
|-------------------------------------------|-----------------------------------|
| DA-20                                     | dimethylhydroxylamine             |
| DA-21                                     | diethylhydroxylamine              |
| DA-22                                     | n-butylhydroxylamine              |
| DA-23                                     | phenylhydroxylamine               |
| DA-24                                     | o-tolylhydroxylamine              |
| DA-25                                     | p-tolylhydroxylamine              |
| DA-26                                     | o-xylylhydroxylamine              |
| DA-27                                     | p-xylylhydroxylamine              |
| DA-28                                     | N,N-di(ethoxyethyl)hydroxylamine  |
| DA-29                                     | N,N-di(methoxyethyl)hydroxylamine |

Hydroxyurea developing agents constitute another preferred class of silver halide developing agents useful in the practice of this invention. Exemplary preferred hydroxyureas are represented by the formula:



wherein R<sup>1</sup>, R<sup>2</sup> and R<sup>3</sup> are hydrogen, alkyl, especially alkyl containing 1 to 4 carbon atoms, such as methyl, ethyl, propyl and butyl, or aryl, typically aryl containing 6 to 10 carbon atoms, such as phenyl, tolyl and xylol. R<sup>1</sup>, R<sup>2</sup> and/or R<sup>3</sup> can contain substituent groups which do not adversely affect developing activity of the described N-hydroxyurea silver halide developing agents. Such substituent groups include, for example, halogen or amino groups. Within the described class of N-hydroxyurea silver halide developing agents especially useful reducing agents are those wherein R<sup>1</sup> is hydrogen, alkyl containing 1 to 4 carbon atoms or aryl containing 6 to 10 carbon atoms, such as phenyl, tolyl or xylol; R<sup>2</sup> is hydrogen, alkyl of 1 to 4 carbon atoms or aryl containing 6 to 10 carbon atoms such as phenyl, tolyl or xylol; R<sup>3</sup> is hydrogen, alkyl containing 1 to 4 carbon atoms or phenyl, tolyl or xylol. Particularly useful hydroxyurea developing agents are those of the formula



wherein R<sup>4</sup> is phenyl, p-methylphenyl, p-methoxyphenyl or p-chlorophenyl. Such developing agents are disclosed in Wilson et al., U.S. Ser. No. 252,036, filed May 10, 1972, commonly assigned. Exemplary preferred hydroxyurea developing agents are set forth below in Table IV.

TABLE IV

| Exemplary Hydroxyurea Developing Agents |                                    |
|-----------------------------------------|------------------------------------|
| DA-30                                   | hydroxyurea                        |
| DA-31                                   | N'-phenyl-N-hydroxyurea            |
| DA-32                                   | N'-(p-tolyl)-N-hydroxyurea         |
| DA-33                                   | N'-(p-methoxyphenyl)-N-hydroxyurea |
| DA-34                                   | N'-(p-chlorophenyl)-N-hydroxyurea  |
| DA-35                                   | N,N'-diphenyl-N-hydroxyurea        |
| DA-36                                   | N'-(m-chlorophenyl)-N-hydroxyurea  |
| DA-37                                   | N'-(p-nitrophenyl)-N-hydroxyurea   |
| DA-38                                   | N',N'-diphenyl-N-hydroxyurea       |
| DA-39                                   | N'-phenyl-N-methyl-N-hydroxyurea   |
| DA-40                                   | N'-ethyl-N-hydroxyurea             |

Another preferred class of developing agents useful in the practice of this invention are pyrimidine developing agents. Particularly preferred pyrimidines are those which in their enol form have adjacent amino and/or hydroxyl ring substituents. Both the amino substituents and the remaining ring positions can be either substituted or unsubstituted, and the substituents, if any, at the 2 and 3 ring positions can, optionally, form a fused ring system. Amino and ring substituents such as alkyl, alkoxy, alkoxyalkyl, alkenyl, aryl, aryloxy, alkaryl, aralkyl, and the like are contemplated. In the preferred form the aliphatic substituent moieties each have 6 or fewer carbon atoms while the aryl substituents are preferably phenyl substituents, but in the 2 and 3 ring positions can be those which form fused rings with the pyrimidine ring. Pyrimidine developing agents of this type are disclosed by Henn and Carpenter in *Photographic Science Engineering*, Vol. 3, at page 135 (1959).

Exemplary preferred pyrimidine developing agents are those set forth below in Table V.

TABLE V

| Exemplary Preferred Pyrimidine Developing Agents |                                                         |
|--------------------------------------------------|---------------------------------------------------------|
| DA-41                                            | 2-isopropyl-4,5,6-trihydroxypyrimidine                  |
| DA-42                                            | 4-amino-5,6-dihydroxy-2-methylpyrimidine                |
| DA-43                                            | 1-methyl-2-propyl-4,5,6-trihydroxypyrimidine            |
| DA-44                                            | 5-aminobarbituric acid (uramyl)                         |
| DA-45                                            | 2,5-diamino-4,6-dihydroxypyrimidine                     |
| DA-46                                            | 2,4,5-triaminopyrimidine                                |
| DA-47                                            | 5-amino-2,4-dihydroxypyrimidine (5-amino-uracil)        |
| DA-48                                            | 5,6-diamino-2,4-dihydroxypyrimidine (5,6-diaminouracil) |
| DA-49                                            | 5-amino-4,6-dihydroxypyrimidine                         |
| DA-50                                            | 6-methyl-2,4,5-trihydroxypyrimidine                     |
| DA-51                                            | 2-amino-4,5-dihydroxypyrimidine                         |

The use of ascorbic acid developing agents is also contemplated. Such developing agents include ascorbic acid, ascorbic acid ketals, and derivatives such as iminoascorbic acids and sugar analogs thereof of the type disclosed by Reynolds in U.S. Pat. 2,688,548, issued Sept. 7, 1954. Exemplary preferred ascorbic acid developing agents of this type are set forth below in Table VI.

TABLE VI

| Exemplary Preferred Ascorbic Acid Developing Agents |                                     |
|-----------------------------------------------------|-------------------------------------|
| DA-52                                               | ascorbic acid                       |
| DA-53                                               | imino-L-erythroascorbic acid        |
| DA-54                                               | imino-L-ascorbic acid               |
| DA-55                                               | imino-D-glucoscorbic acid           |
| DA-56                                               | imino-6-desoxy-L-ascorbic acid      |
| DA-57                                               | imino-L-rhamnoscorbic acid          |
| DA-58                                               | imino-L-fucoscorbic acid            |
| DA-59                                               | imino-D-glucosheptoscorbic acid     |
| DA-60                                               | imino-sorboascorbic acid            |
| DA-61                                               | imino- $\omega$ -lactoascorbic acid |
| DA-62                                               | imino-maltoascorbic acid            |
| DA-63                                               | imino-L-araboscorbic acid           |
| DA-64                                               | imino-D-glucoscorbic acid           |
| DA-65                                               | imino-D-galatoscorbic acid          |
| DA-66                                               | imino-L-glucoscorbic acid           |
| DA-67                                               | imino-L-alloscorbic acid            |

The photographic silver halide developers of my invention employ the developing agents singly or in combination in concentrations of from 0.01 molar to saturation, preferably in concentrations of from 0.01 to 0.5 molar. Except for the inclusion of ruthenium complexes and the selection of the developing agents, the photographic developers are otherwise of conventional composition. They typically include water as a solvent and are rendered basic by the inclusion of a suitable basic material. Typical photographic developers useful in the practice of this invention exhibit a pH in the range from about 9 to about 13. Typically one or a combination of alkali metal hydroxides and salts, such as sodium or potassium hydroxide, carbonate, bicarbonate, phosphate, silicate or the like, are employed to maintain the desired degree of basicity. To reduce oxidation of the developing agents present stabilizers, such as alkali metal and amine sulfites, are typically incorporated in a concentration of from 0.001 to 10 molar, as is well understood in the art.

Other conventional photographic silver halide developer addenda can, of course, be incorporated to produce known effects. Where a hydroquinone is employed as the developing agent and it is desired to develop photographic films of high contrast, such as those employed in the graphic arts—i.e., so called lith-type films, it is preferred to incorporate into the developer a carbonyl bisulfite-amine condensation product and at least about 0.075 mole of free amine per liter of developer composition, as taught by Masseth U.S. Pat. 3,573,914, issued Apr. 6, 1971. Such addenda stabilize the developer and eliminate drag streaks and dot distortions typically associated with machine processing.

The carbonyl bisulfite-amine condensation products are preferably formaldehyde bisulfite-amine condensation products such as

sodium-2-hydroxyethylaminomethane sulfonate,  
sodium-2-hydroxypropylaminomethane sulfonate,  
sodium-1,1-dimethyl-2-hydroxylaminomethane sulfonate,  
sodium-1,1-bis(hydroxymethyl)ethylaminomethane sulfonate,  
sodium-tris(hydroxymethyl)methylaminomethane sulfonate,  
sodium-3-hydroxypropylaminomethane sulfonate,  
sodium-bis(2-hydroxyethyl)aminomethane sulfonate,  
sodium-N,N-bis(2[1-hydroxy]propyl) aminomethane sulfonate,

sodium-N-isopropyl-N-(2-hydroxyethyl)-aminethane sulfonate, sodium-N-ethyl-N-(2-hydroxyethyl)-aminomethane sulfonate, and sodium-N-methyl-N-(2-hydroxyethyl)-aminomethane sulfonate.

The carbonyl bisulfite-amine condensation products can be used alone or in any combination and can be employed in any combination which is effective to provide a low level of sulfite ion for the developer composition. A suitable concentration for the carbonyl bisulfite-amine condensation product is from about 0.1 to about 1.0 mole per liter of liquid developer composition and is preferably from about 0.25 to about 0.50 mole per liter of liquid developer composition.

The carbonyl bisulfite-amine condensation product can be added to the developer composition as a separate compound or formed in situ. Methods for preparing these compounds are disclosed, for example, in U.S. Pat. 2,388,816 of Bean issued Nov. 13, 1945. It is meant to include within the definition of carbonyl bisulfite-amine condensation product either the compound itself or the individual components which form the compound in situ.

The free or uncombined amine compounds which can be employed include primary and secondary amines such as

2-aminoethanol,  
1-amino-2-propanol,  
2-amino-  
2-amino-2-methyl-1,3-propanediol,  
2-amino-2(hydroxymethyl)-1,3-propanediol,  
3-amino-1-propanol,  
2,2'-iminodiethanol,  
di-iso-propanolamine,  
2-isopropylaminoethanol,  
2-ethylaminoethanol,  
2-methylaminoethanol, etc.

These amines can be used alone or in any combination and should be employed in a concentration of at least about 0.075 mole per liter of developer composition. Concentrations of the amine below this minimum value do not provide a stable developer. A suitable range of concentrations for the amine compound is from about 0.075 to about 3.0 moles per liter of developer composition and is preferably from about 0.20 to about 9.0 mole per liter of developer composition. The free amine present in the developer composition can be the same amine used to prepare the carbonyl bisulfite-amine condensation product or it can be a different amine.

While I have disclosed my invention in terms of the basic aqueous photographic developers used to develop silver halide photographic elements, it is apparent that my invention can take the form of compositions useful in forming these photographic developers.

It is generally well within the capabilities of the photographic processor to add to water the ingredients necessary to constitute a basic aqueous photographic developer, once directions have been supplied. It is accordingly common practice to package and sell compositions which, when added to water or aqueous solutions alone or in combination with other materials, will form a useful photographic developer.

In one form of my invention I contemplate a composition consisting essentially of the developing agents and the ruthenium complexes described above as useful in the practice of my invention. Since the ingredients used to form the photographic developers of my invention are generally compatible when stored together in the absence of a solvent, I prefer in most instances to form a composition which includes in addition to the ruthenium complexes and the developing agents of my invention all other ingredients which, when added to water, form a photographic developer

according to my invention. Where one or more of these ingredients prove chemically incompatible or otherwise disadvantageous to package with the other ingredients, they can, of course, be packaged separately.

In a preferred composition for forming a photographic developer the ruthenium complexes and developing agents can be present in the relative proportions desired in the photographic developer—e.g., from 0.2 to  $1 \times 10^{-5}$  moles of ruthenium complex per mole of developing agent. These proportions are not required, however, since additional developing agent or ruthenium complex can be supplied to the photographic developer from a separate source. In like manner remaining ingredients for the photographic developer can be present in various proportions, preferably in the proportion desired in the photographic developer.

My invention may be further appreciated by reference to the following specific examples.

#### Examples 1 through 11 — Acceleration of Induction Periods

A number of representative developing agents were chosen and separately employed to form photographic silver halide developer compositions consisting essentially of 200 ml of water, 20 grams of sodium sulfite, 10 g of sodium carbonate, sufficient acetic acid to reduce the pH of the developer to the desired value and a 0.05 molar concentration of the developing agent. Each developer was then divided into two aliquot portions and a  $5 \times 10^{-4}$  molar concentration of hexammine ruthenium (III) chloride (RU-1a) was added to one aliquot portion. Induction periods were then determined employing the procedures of Willis and Pontius, cited above. A black-and-white photographic motion picture print film bearing a fine grain silver chlorobromide emulsion coating was exposed and developed. The results are summarized in Table VII below.

TABLE VII

| Example No. | Developing Agents                               | Comparative Induction Periods |                                           | Induction Period (seconds)<br>w/o Ru(III) | w Ru(III) |
|-------------|-------------------------------------------------|-------------------------------|-------------------------------------------|-------------------------------------------|-----------|
|             |                                                 | pH                            | Induction Period (seconds)<br>w/o Ru(III) |                                           |           |
| Control     | Elon*(N-methyl-p-aminophenol sulfate)           | 10.0                          | 1.0                                       | 1.0                                       | 1.0       |
| Control     | p-aminophenol                                   | 10.0                          | 1.5                                       | 1.5                                       | 1.5       |
| Control     | 2,4-diaminophenol dihydrochloride               | 7.2                           | 1.5                                       | 1.5                                       | 1.5       |
| Control     | hydroquinone-Elon (equal pts. by wt.)           | 9.5                           | 11.0                                      | 9.0                                       | 35.0      |
| Control     | hydroquinone-Elon (4:2 pts. by wt.)             | 9.0                           | 31.0                                      | 35.0                                      | 35.0      |
| Control     | 1-phenyl-3-pyrazolidone                         | 12.0                          | ~0.0                                      | ~0.0                                      | ~0.0      |
| Control     | dihydroanhydroperidinohexose reductone          | 11.6                          | ~0.0                                      | ~0.0                                      | ~0.0      |
| Control     | N,N-diethyl-p-phenylenediamine                  | 12.0                          | 2.0                                       | 7.0                                       | 7.0       |
| Control     | 4-amino-N-ethyl-N-( $\beta$ -methanesulfonamido |                               |                                           |                                           |           |

TABLE VII-continued

| Example No. | Developing Agents                                                 | Comparative Induction Periods |       | Induction Period (seconds)<br>w/o Ru(III) | Induction Period (seconds)<br>w Ru(III) |
|-------------|-------------------------------------------------------------------|-------------------------------|-------|-------------------------------------------|-----------------------------------------|
|             |                                                                   | pH                            |       |                                           |                                         |
| Control     | ethyl-m-toluidine sesquisulfate                                   | 11.7                          |       | ~0.0                                      | ~0.0                                    |
| 1           | 4-amino-3-methyl-N-ethyl-N-β-methoxyethylaniline p-tolylsulfonate | 10.5                          | 10.0  | 10.0                                      |                                         |
| 2           | ascorbic acid (DA-52)                                             | 10.0                          | 90.0  | 6.0                                       |                                         |
| 3           | hydroquinone (DA-6)                                               | 10.0                          | 30.0  | 5.0                                       |                                         |
| 4           | methylhydroquinone (DA-11)                                        | 10.0                          | 130.0 | 11.0                                      |                                         |
| 5           | pyrogallol (DA-4)                                                 | 10.0                          | 9.0   | 1.0                                       |                                         |
| 6           | 2,5-dichlorohydroquinone                                          | 10.0                          | 10.0  | 1.0                                       |                                         |
| 7           | 2-isopropyl-4,5,6-trihydroxypyrimidine (DA-41)                    | 11.8                          | 22.0  | ~0.0                                      |                                         |
| 8           | 4-amino-5,6-dihydroxy-2-methylpyrimidine (DA-42)                  | 11.0                          | 11.0  | ~0.0                                      |                                         |
| 9           | 1-methyl-2-propyl-4,5,6-trihydroxypyrimidine (DA-43)              | 11.5                          | 10.0  | ~0.0                                      |                                         |
| 10          | N-(p-methoxyphenyl)-N'-hydroxyurea (DA-33)                        | 12.0                          | 72.0  | 8.0                                       |                                         |
| 11          | N-(p-chlorophenyl)-N'-hydroxyurea (DA-34)                         | 12.3                          | 55.0  | 1.0                                       |                                         |
|             | diethylhydroxylamine (DA-21)                                      | 12.1                          | 117.0 | 10.0                                      |                                         |

\*Trademark of Eastman Kodak Company

In reviewing the results of Table VII it is apparent that all of the photographic silver halide developer compositions incorporating the ruthenium complex and employing developing agents according to my invention exhibited marked reductions in induction periods attributable to the incorporation of the ruthenium (III) complex. Only one of the photographic developers incorporating a developing agent (Elon) having an induction period of less than 5 seconds exhibited any reduction in the induction period attributable to the incorporation of the ruthenium (III) complex. However, the reduction of the induction period was quite small as compared to the induction period reductions exhibited by the photographic developers of my invention. Only one of the developing agents (4-amino-3-methyl-N-ethyl-N-β-methoxyethylaniline p-tolylsulfonate) exhibiting an induction period of more than 5 seconds in the absence of the ruthenium (III) complex failed to show marked reduction of the induction period as a result of incorporating the ruthenium (III) complex. This lack of induction period reduction was attributed to the fact that this particular developing agent, like the p-aminophenols and p-phenylenediamines in general, more readily reduces silver halide than the ruthenium (III) complex.

#### Examples 12 through 15 — Acceleration on Continuation Stage

Employing the procedures of Willis and Pontius, cited above, the acceleration of the continuation stage was measured for some of the developers of Examples 1 through 11. The acceleration of the continuation stage is reported as the ratio of the development rate with the ruthenium (III) complex divided by the development rate without the ruthenium (III) complex. Similarly, induction period accelerations reported in subsequent examples represent a ratio of the induction period without the ruthenium complex divided by the induction period with the ruthenium complex present. Thus acceleration values are above 1.0 when development was accelerated and below 1.0 when development was retarded. The results are summarized below in Table VIII.

Table VIII

| Example No. | Developing Agent | Acceleration of Continuation Stage |
|-------------|------------------|------------------------------------|
| Control     | Elon             | 1.0                                |

Table VIII-continued

| Example No. | Developing Agent                                  | Acceleration of Continuation Stage |
|-------------|---------------------------------------------------|------------------------------------|
| Control     | p-aminophenol                                     | 1.0                                |
| Control     | 4-amino-3-methyl-N-ethyl-N-β-methoxyethyl aniline | 0.86                               |
| 12          | pyrogallol (DA-4)                                 | 2.4                                |
| 13          | hydroquinone (DA-6)                               | 2.3                                |
| 14          | ascorbic acid (DA-52)                             | 2.9                                |
| 15          | methylhydroquinone (DA-11)                        | 8.9                                |

#### Examples 16 through 18 — Comparison of Development and Ruthenium Reduction Rates

A 0.1 molar solution of sodium carbonate in water and a 3.0 molar sodium bicarbonate aqueous solution were mixed to obtain a pH of 10. Hexammine ruthenium(III) chloride was then added to the solution to produce a net optical density upon standing of 0.1. At the same time a developing agent and sodium sulfite were each added to water to a concentration of 0.01 molar to form a second solution. The solutions were then mixed together and the rate of density loss was immediately measured spectrophotometrically. From this measurement the rate of ruthenium(III) complex reduction to the corresponding colorless ruthenium(II) complex was calculated. The rates of silver halide development exhibited by the developing agents in the absence of the ruthenium(III) complex were determined using the photographic elements and developers lacking a ruthenium complex of Examples 1 through 11. Rates are reported in units of liter mole<sup>-1</sup> second<sup>-1</sup>. The results are summarized below in Table IX.

TABLE IX

| Example No. | Developing Agent           | Exemplary Comparative Reduction Rates |         |
|-------------|----------------------------|---------------------------------------|---------|
|             |                            | Silver Halide                         | Ru(III) |
| 16          | hydroquinone (DA-6)        | 0.16                                  | 1.1     |
| 17          | methylhydroquinone (DA-11) | 0.046                                 | 2.7     |
| Control     | Elon                       | 0.46                                  | 0.27    |
| Control     | p-aminophenol              | 0.18                                  | 0.11    |
| 18          | ascorbic acid (DA-52)      | 0.05                                  | 0.8     |

Table IX illustrates that the developing agents, such as hydroquinone and ascorbic acid developing agents,

useful in the practice of my invention, exhibit reduction rates for ruthenium(III) which are markedly greater than their reduction rates for silver halide. At the same time, the aminophenol developing agents exhibit rates of reduction of silver halide which are somewhat greater than their rates of reduction of ruthenium(III). This is in agreement with the observation that the induction periods of p-aminophenols are not reduced through the use of ruthenium(III) complexes as development accelerators.

The examples which follow show the effectiveness of additional ruthenium(II) and (III) cationic complexes as development accelerators.

#### Example 19

The procedures of Examples 1 through 15 were repeated using hydroquinone (DA-6) as a developing agent and tris(2,2'-bipyridine) ruthenium(III) chloride (RU-62a) as a development accelerator. An induction period acceleration of 4 and a continuation stage acceleration of 2 was observed. Because of the potential relationships of the silver chlorobromide and the development accelerators it is not believed that the development accelerator was functioning in this situation to form a redox couple between the developing agent and silver halide.

#### Example 20

The procedure of Example 19 was repeated, but with the substitution of tris(ethylenediamine)ruthenium(II) tetrabromozincate (RU-12thiocyanatopentammine. An induction period acceleration of 60 and a continuation stage acceleration of 1.25 was observed.

#### Examples 21 through 23

The procedure of Examples 1 through 11 was repeated, but with the substitution of thiocyaanatopentammine ruthenium(III) methylsulfonate for the hexammine ruthenium(III) chloride. The results are summarized below in Table X.

TABLE X

| Example No. | Developing Agent   | Induction Period Acceleration |
|-------------|--------------------|-------------------------------|
| Control     | p-aminophenol      | 0.86                          |
| Control     | Elon               | 1.0                           |
| 21          | hydroquinone       | 29.0                          |
| 22          | methylhydroquinone | 8.5                           |
| 23          | ascorbic acid      | 9.8                           |

The invention has been described with particular reference to preferred embodiments thereof but it will be understood that variations and modifications can be effected within the spirit and scope of the invention.

I claim:

1. A composition useful in developing silver halide photographic elements comprising at least one silver halide developing agent and a development accelerating amount of at least one ruthenium(III) or (II) cationic complex including at least four ligands chosen from the class consisting of ammine or amine ligands, each said developing agent exhibiting in the absence of other silver halide developing agents and said ruthenium complex a silver halide development induction period in excess of 5 seconds and

at least one said developing agent exhibiting a rate of reduction of ruthenium(III) in said ruthenium(III) cationic complex, or produced by the oxidation of said ruthenium(II) cationic complex, which exceeds its rate of reduction of silver halide.

2. A composition according to claim 1, in which said ruthenium complex includes at least four ammine ligands.
3. A composition according to claim 1, in which said ruthenium complex is a hexammine ruthenium(II) or hexammine ruthenium(III) complex.
4. A composition according to claim 1, in which said ruthenium complex includes at least four amine ligands.
5. A composition according to claim 4, in which said amine ligands are alkylene diamine ligands in which said alkylene group has from 1 to 6 carbon atoms.
6. A composition according to claim 5, in which said ruthenium complex is a tris(ethylenediamine)ruthenium(II) or tris(ethylenediamine)ruthenium(III) complex.
7. A composition according to claim 4 in which said amine ligands are pyridine ligands.
8. A composition according to claim 7 in which said ruthenium complex is a tris(2,2'-bipyridine)ruthenium(II) or tris(2,2'-bipyridine)ruthenium(III) complex.
9. A composition according to claim 1, in which said ruthenium(III) complex exhibits a reduction potential which is no less positive than the oxidation potential of said developing agent.
10. A composition according to claim 9 in which said ruthenium(III) complex exhibits a reduction potential which is between the oxidation potential of the developing agent and the reduction potential of silver halide.
11. A composition according to claim 1, in which said developing agent is chosen from the group consisting of polyhydroxybenzene, ascorbic acid, hydroxylamine, hydroxyurea and pyrimidine developing agents as well as mixtures thereof.
12. A basic aqueous photographic developer containing a development accelerator and as the sole developing agent or agents one or more developing agents chosen from the class consisting of polyhydroxybenzene, ascorbic acid, hydroxylamine, hydroxyurea and pyrimidine developing agents, wherein the improvement comprises from  $1 \times 10^5$  to 0.1 mole per liter of developer of at least one ruthenium(II) or ruthenium(III) complex development accelerator including at least four ligands chosen from the class consisting of ammine or amine ligands, the reduction potential of said ruthenium(III) complex or the ruthenium(III) complex produced by oxidation of said ruthenium(II) complex more positive when the oxidation potential of at least one of said developing agents.
13. A basic photographic developer according to claim 12 comprised of the further improvement in which a hydroquinone polyhydroxybenzene developing agent chosen from said class of developing agents is present.
14. A basic photographic developer according to claim 13 comprised of the further improvement in which said hydroquinone includes at least one halogen or alkyl substituent, said alkyl substituent having from 1 to 6 carbon atoms.
15. A basic photographic developer according to claim 12 comprised of the further improvement in which a pyrogallol polyhydroxybenzene developing

agent chosen from said class of developing agents is present.

16. A basic photographic developer according to claim 12 comprised of the further improvement in which a catechol polyhydroxybenzene developing agent chosen from said class of developing agents is present.

17. A basic photographic developer according to claim 12 comprised of the further improvement in which a pyrimidine developing agent is present having in the enol form adjacent ring substituents chosen from the class consisting of amino and hydroxyl substituents.

18. A basic photographic developer according to claim 12 comprised of the further improvement in which said ruthenium complex includes at least four ammine ligands.

19. A basic photographic developer according to claim 18 comprised of the further improvement in which said ruthenium complex is a hexammine ruthenium(II) or hexammine ruthenium(III) complex.

20. A basic aqueous photographic developer containing a development accelerator and hydroquinone as the sole developing agent, wherein the improvement comprises

from  $1 \times 10^{-5}$  to 0.1 mole per liter of developer of a hexammine ruthenium(II) or hexammine ruthenium(III) complex.

21. A method of accelerating the development of an imagewise exposed silver halide photographic element in a developer composition containing at least one silver halide developing agent, which method comprises

incorporating in the developer composition a development accelerating amount of at least one ruthenium(III) or (II) cationic complex including at least four ligands chosen from the class consisting of ammine or amine ligands,

each developing agent exhibiting in the absence of other silver halide developing agents and the ruthenium cationic complex an induction period in excess of 5 seconds and

5

10

15

20

25

30

35

40

45

50

60

65

at least one developing agent in the developer composition exhibiting a rate of reduction of ruthenium(III) in the ruthenium(III) cationic complex, or produced by the oxidation of the ruthenium(II) cationic complex, which exceeds its rate of reduction of silver halide, and

bringing the developer composition into contact with the imagewise exposed photographic element.

22. A method of accelerating the development of an imagewise exposed silver halide photographic element in a developer composition containing as the sole developing agent or agents one or more developing agents chosen from the class consisting of polyhydroxybenzene, ascorbic acid, hydroxylamine, hydroxyurea and pyrimidine developing agents, which method comprises

incorporating in the developer composition from  $1 \times 10^{-5}$  to 0.1 mole per liter of developer of at least one ruthenium(II) or ruthenium(III) complex including at least four ligands chosen from the class consisting of ammine or amine ligands, the reduction potential of the ruthenium(III) complex or the ruthenium(II) complex produced by oxidation of the ruthenium(II) complex being more positive than the oxidation potential of at least one of the developing agents, and

bringing the developer composition into contact with the imagewise exposed photographic element.

23. A method according to claim 22 including the step of incorporating hexammine ruthenium(II) or hexammine ruthenium(III) complex.

24. A method of accelerating the development of an imagewise exposed silver halide photographic element in a developer composition containing as the sole silver halide developing agent a hydroquinone, which method comprises

incorporating in the developer composition from  $1 \times 10^{-5}$  to 0.1 mole per liter of developer of a hexammine ruthenium(II) or hexammine ruthenium(III) complex and

bringing the developer composition into contact with the imagewise exposed photographic element.

\* \* \* \* \*

55